

March 14, 1933.

W. S. SMITH ET AL

1,901,005

MANUFACTURE OF LOADED ELECTRIC SIGNALING CONDUCTORS

Filed May 25, 1931

Fig. 1.



Fig. 2.



Inventors:

W. S. Smith,

H. J. Garnett,

J. N. Dean;

By their Attorneys,

Frederick Wright

## UNITED STATES PATENT OFFICE

WILLOUGHBY STATHAM SMITH, OF BENCHAMS, NEWTON POPPLEFORD, HENRY JOSEPH GARNETT, OF LYMNE, SOLEFIELDS, SEVENOAKS, AND JOHN NORMAN DEAN, OF ORPINGTON, ENGLAND

## MANUFACTURE OF LOADED ELECTRIC SIGNALING CONDUCTORS

Application filed May 25, 1931, Serial No. 539,964, and in Great Britain February 14, 1931.

This invention relates to improvements in the manufacture of loaded electric signaling conductors, and more particularly to conductors loaded with a wire or tape of magnetic material wound upon the conductor.

Such conductors are usually subjected to an annealing treatment in order to develop magnetic permeability in the loading. After winding on to the conductor the loading tape or wire, the latter, even after annealing, tends to grip very tightly the conductor with the result that the magnetic properties are apt not to be fully developed.

To overcome this strained condition of the loading tape it is the practice to employ what is known as a "spacer" between the loading tape or wire and the conductor, which spacer is removed during the subsequent annealing operation.

Various forms of spacer have been proposed, but up to the present all those which are of a carbonaceous nature, such for example as a paper tape or a combustible thread, have not proved satisfactory owing to the deposits of carbon which are formed in the annealing furnace.

The object of the present invention is to overcome these objections to the use of a carbonaceous spacer by removing the carbon deposit.

Experiments have been made with oxygen, which has been introduced in controlled proportions with the inert gas into the annealing furnace with the object of reacting with the carbon and other reducing bodies that may be present. It has however proved practically impossible to control the inlet of oxygen so that the reducing bodies are fully oxidized while at the same time the conductor is unattacked by the oxygen.

According to the present invention conductors having a spacer of a carbonaceous nature, are treated in an atmosphere containing a gas, such as water vapor containing combined oxygen, which oxygen is capable of reacting at the temperature of the annealing operation with the carbon or other reducing bodies formed.

An atmosphere consisting of an inert gas e. g. nitrogen admixed with water vapor

has proved satisfactory. At the high temperature the water vapor probably oxidizes the carbon in accordance with the equation



and indeed carbon monoxide has been detected in the gases issuing from the tube at the end where the conductor leaves the furnace.

The proportion of water vapor admixed with e. g. the nitrogen does not seem to be at all critical provided sufficient water is present to oxidize the carbon to carbon monoxide. Loaded conductors have been successfully heat-treated in an atmosphere consisting almost entirely of water-vapor. The nickel alloy loading material of the conductor is substantially unaffected when it has been heat-treated in an atmosphere containing only a relatively small or moderate proportion of water-vapor, but is covered with a very thin film, probably of oxide, when high proportions of water vapor are used in the gaseous mixture. Although the presence of this thin film is harmless in the case of conductors loaded with comparatively thick tape, e. g. .006 inch thick, it is preferable when very thin tape e. g. only .001 inch thick is used, to employ such a proportion of water vapor that no oxidation of the metal surface occurs.

The water may be introduced either in the form of steam or as drops of liquid water through a special entrance tube into the furnace or it may be sprayed in with the nitrogen.

As has been stated above, the gases issuing from the end of the furnace tube contain carbon monoxide, the highly poisonous nature of which is well known. In order to prevent this gas escaping into the air of the room, an adapter is attached to the exit end of the furnace tube, which adapter may be made of copper, brass, gun-metal or any suitable material. Two forms of adapters are illustrated in Figures 1 and 2 of the accompanying drawing which are sectional views.

The adapter may consist of a length of tubing 1 having a tapered bore 2 which is

55

60

65

70

75

80

85

90

95

100

attached to the heating tube indicated at 3 so as to restrict for a considerable distance that mouth of the heating tube through which the conductor leaves the furnace, this 5 tapered portion of the tube fitting the conductor fairly closely.

A branch pipe 4 to which a suction pump (not shown) is attached, is fitted to the heating tube at or adjacent the beginning of the 10 restricted portion.

The carbon monoxide and other gases from the furnace are drawn off by the suction pump through the branch pipe 4 and are prevented from escaping into the air 15 of the room by the steady intake of air (indicated by the arrows *a*) drawn in by the action of the pump through the narrow opening round the emerging conductor. As this causes a vacuum in the tube with con- 20 sequent intake of air at the lead in end together with the nitrogen and steam, it is better to provide a partition in the heating tube so as to form a separate chamber at the exit end and to control the pressure in this 25 chamber so that it is only just below that of the atmosphere. Such an arrangement is shown in Figure 2 in which the adapter consists of a cylindrical container 5 having axial holes 6 for the passage of the con- 30 ductor. 7 and 8 are inlet and outlet pipes connected to the chamber 9 of container 5.

Alternatively a controlled amount of air or oxygen may be admitted into the furnace tube at the end of the hot zone, suffi- 35 cient to oxidize the reducing gases such as carbon monoxide, hydrocarbons (if present) and hydrogen, to carbon dioxide and water. The disadvantage of this method is that it is difficult so to adjust the amount of air or 40 oxygen admitted that the reducing gases are completely oxidized while the heated conductor is unattacked by the oxygen.

What we claim is:—

1. In the manufacture of a loaded signal 45 conductor having a spacing material applied between the central conductor and the loading material, wherein said spacing material is removed during the process of heat treating the conductor in order to pro- 50 vide a space between the conductor and the loading material retaining a carbonaceous material, the method of subjecting said carbonaceous material to an inert atmosphere containing water vapour, which water 55 vapour reacts at the temperature of the heat treatment with the retained carbonaceous material for preventing attack of said carbonaceous material upon said conductor.

2. In the manufacture of a loaded signal 60 conductor having a carbonaceous material applied between the central conductor and the loading material, wherein said carbonaceous material is removed during the process of heat treating the conductor in 65 order to provide a space between the con-

ductor and the loading material while leaving a carbon residue, the method of sub- 70 jecting said carbon residue to an atmosphere consisting of a mixture of nitrogen and water vapour for the purpose of dissipating said carbon residue and preventing the at- tack thereof upon said conductor.

In testimony that we claim the foregoing 75 as our invention, we have signed our names this 12th day of May, 1931.

WILLOUGHBY STATHAM SMITH.

HENRY JOSEPH GARNETT.

JOHN NORMAN DEAN.

80

85

90

95

100

105

110

115

120

125

130